# EUROPEAN PATENT APPLICATION

(11) **EP 0 684 092 A1**
(43) Date of publication of application: **29.11.1995**
(21) Application number: 94925051.8
(22) Date of filing: 05.08.1994
(51) Int. Cl.: B21C 37/04

(54) **METHOD OF MANUFACTURING WIRE**

(30) Priority: 07.09.1993 RU 93044098
(71) Applicant: Aktsionernoe Obschedtvo Zakrytogo Tipa "Bimet-Nytva", Kirov, 610016 (RU)
(72) Inventor: STAZAEV, Vladimir Nikolaevich, Kirov, 610000 (RU)
(74) Representative: Lins, Edgar, Dipl.-Phys. Dr.jur.
(86) International application number: RU9400185
(87) International publication number: WO9507155

(57) **Abstract**

A half-finished product for wire drawing is obtained by cutting ribbon-like material into narrow rectangular strips, welding the strips together and rounding the edges.

## Description

### Technical Field

The present invention relates to wire production practice.

### Background Art

Known in the present state of the art is a method for producing a long-length wire rod by drawing a bar through drawing dies until a preset size is obtained (cf. British Patent # 1,400,872, Int. Cl. B 21 C 37/04, 1975).

The process in question is a labor-consuming one, since it involves special equipment for wire drawing through drawing dies for a number of passes.

According to USSR Patent # 683,606, Int.Cl. B 21 C 37/04, 1979, a less number of a bar drawing passes are required to obtain a required rod dimension, since the bar is preliminarily given a polyhedral cross-sectional shape having the dimensions to a maximum extent approximating the preset wire rod dimensions.

### Disclosure of the Invention

The present invention has for its principal object to provide a higher output of the wire production process and a lower power and material consumption.

The foregoing object is accomplished due to producing a a wire bar by cutting a strip rolled stock into narrow strips, rounding-off the edges of the strips using the etching process or mechanically, and drawing the resultant wire bar through drawing dies until a preset dimension is obtained. Preparatory to drawing the wire bars are butt-welded together.

### Embodiments of the Invention

The herein-proposed method is carried into effect as follows.

To produce dia.1 mm copper wire (from M-3 alloy), a 1.5-mm-thick strip rolled stock is produced on double-stand rolling mills, the rolling process occurring for five passes at a speed of 2 - 3.5 m/s and a 20% reduction per pass.

Then the strip rolled stock is cut into 1.5-mm-wide strips to obtain a square wire bar having a 1.5 x 1.5 mm cross-section.

Next the ends of the resultant wire bars are butt-welded together, whereupon the edges of the resultant long-length bar are rounded off by the edging process.

The final operation, i.e., drawing is performed for three passes at a drawing speed of 0.5 m/s and a 17% reduction per pass.

To produce dia.0.75 mm brass wire a strip stock is rolled for six passes to a thickness of 1 mm, the rolling conditions being the same as in producing copper wire.

The strip stock is cut into 1-mm-wide strips, which are then welded together, the edges are rounded off, and the strips are drawn to a diameter of 0.75 mm for three passes, the reduction per pass being 8%.

## Claims

1. A method for wire producing, consisting in that wire bars are obtained and then drawn to a required dimension, CHARACTERIZED in that said wire bars are produced by cutting strip rolled stock into rectangular-cross-section strips and rounding-off the edges thereof.

2. A method according to Claim 1, CHARACTERIZED in that preparatory to rounding-off the edges of the rectangular-cross-section strips they are butt-welded together.

3. A method according to Claims 1 and 2, CHARACTERIZED in that the edges are rounded off by the etching process.
